

No. 10,574.

PATENTED FEB. 28, 1854.

J. RENTON.  
ZINC WHITE FURNACE.

Fig. 2.



Fig. 3.



Fig. 4.

Fig. 1.



# UNITED STATES PATENT OFFICE.

JAMES RENTON, OF NEWARK, NEW JERSEY.

## IMPROVEMENT IN ZINC-WHITE FURNACES.

Specification forming part of Letters Patent No. **10,574**, dated February 28, 1854.

*To all whom it may concern:*

Be it known that I, JAMES RENTON, of Newark, in the county of Essex and State of New Jersey, have invented certain new and useful Improvements in Apparatus for Manufacturing Metallic Zinc and the Oxide of Zinc; and I do hereby declare that the following is a full, clear, and exact description of the same, reference being had to the accompanying drawings, forming part of this specification, in which—

Figure 1 is a longitudinal vertical section taken through the center of the apparatus. Fig. 2 is a transverse vertical section in the line \* \* of Fig. 1. Fig. 3 is a longitudinal vertical section in the line \* \* of Fig. 2. Fig. 4 is a horizontal section.

Similar letters of reference indicate corresponding parts in each of the several figures.

The apparatus which forms the subject of this invention is principally intended to carry out a new mode of manufacturing the oxide of zinc and metallic zinc; but it possesses another important feature in affording facilities for the treatment of the residuum of the ore, when that residuum is of value. The present mode of manufacturing the oxide of zinc, which is attended with many difficulties and much labor and expense, is to place the pulverized zinc ores in a horizontal furnace, protected from the gases of the fuel by fire-brick below and above. The ore in this furnace requires frequent stirring. The process is rendered very tedious and expensive by reason of the small charge of ore that each furnace can operate upon at once, and the great delay caused by the time required to cool the furnace sufficiently to discharge its contents and recharge it again. The production of metallic zinc requires another and separate operation necessarily expensive. One object of my invention is to obviate these serious defects both in the manufacture of zinc oxide and zinc metal by producing them both at one continuous operation, and much more rapidly and at a large saving in cost. Another object is to afford convenience for the treatment, when desirable, of the residuum of certain ores of zinc—as, for instance, the ore found in the State of New Jersey, known as “franklinite zinc ore,” which contains a portion of iron. My apparatus, when combined with a

puddling furnace, will produce oxide of zinc, or both oxide and metallic zinc, and at the same operation wrought-iron from the above ore.

I will now proceed to describe the construction and operation of my apparatus.

The accompanying drawings represent it as specially constructed for the manufacture of zinc from the franklinite ore, and intended to be combined with an iron-puddling furnace, to be heated by the waste heat therefrom; but this serves to illustrate the invention fully, as when other ores are employed the only essential difference will be in the arrangement of the furnace or fire and in the means of discharging the apparatus of the residuum after the zinc is extracted, which may be such as is most convenient.

D is a chamber intended to be placed over the preparatory bottom B of the puddling-furnace, and to be heated by the waste heat of the said furnace passing through it to the chimney.

F F are two series of vertical tubes, which are placed or built in the middle of the chamber D at a short distance apart, and have the whole of their outer sides exposed to the heat, but are sheltered on their inner sides. These tubes receive the ore on the inner side of each ore-tube, F, or that side sheltered from the heat. There are openings f f, similar to what are known as “lower openings,” at short distances apart in vertical rows, commencing some distance above the bottom, and terminating near the top of the tube, and the space between the tubes is divided by partitions g g, extending from the bottom nearly to the top into a number of tubes, M M. The lower part of the space between the ore-tubes F F is undivided, as the partitions g g do not extend to the bottom, and it is furnished with a spout, h, which is closed by a suitable shutter. Each row of ore-tubes F is furnished at the bottom with ore-spouts b b and slides c c, for controlling the discharge of the ore. The tubes F F and M M are all covered by a hood or trunk, N, which has openings at the sides, which serve for the purpose of charging the tubes, and also for the admission of air to the trunk, which is also provided with openings j and k, one at each end. The tubes M M are furnished at the top with a sliding shutter, l, (shown only

in Fig. 2,) which is for the purpose of closing them.

The ore previously to being submitted to the operation of the apparatus is pulverized and mixed with such a percentage of carbon as may be deemed advisable. The ore-tubes F F are filled, and the fuel in the fire-chamber then ignited. The heat and gases from the fuel, after passing over the hearth of the puddling-furnace, pass into the chamber D, giving to the tubes and the ore therein, which is protected from the gases, the proper degree of heat to set free from the ore all the volatile matter which escapes through the openings f f into the spaces M M. When the shutter l at the top of the said spaces M M is left open, the volatile matter escapes into the trunk N, and carried off with cold drafts of air, which are admitted to the trunk through its openings, to any suitable receptacle placed in communication with the trunk, and condensed into the oxide of zinc; but when it is desired to produce zinc in metallic form, the spaces M M are closed at the top by the slide l and the spout h is opened. The volatile matter from the ore is then condensed in the center space in the form of metallic zinc, which will run out at the spout h into any suitable receptacle. Though the greater portion of the vapor from the ore will escape through the openings f f, still a certain portion will always escape at the top of the tubes F F. This portion, whether the slide l is closed or open, escapes into the trunk N, and is converted into oxide of zinc. Thus, when the slide l is closed, zinc metal and the oxide of zinc are at the same time formed.

I have now shown that the oxide of zinc alone, or oxide of zinc and zinc metal, can be at the same time produced. The proportionate quantities of oxide of zinc and metallic zinc which may be produced may, to a certain extent, be controlled by opening one, two, or more of the tubes F F at the top. When all the volatile matter is extracted from the ore, the residuum, according to its nature, is discharged by opening the slides e e onto the puddling-hearth, to be there treated for the manufacture of wrought-iron, or into any receptacle suitable to receive it for future treatment, and a new charge is placed in the ore-tubes. While the new charge of ore is having the volatile portion set free and extracted,

the residuum of the last charge may be subjected to the necessary treatment on the hearth, or other receptacle below the chamber D. This apparatus may also be employed in the collection and manufacture of other volatile matters contained in ores.

The great advantage derived from my invention in the manufacture of oxide of zinc and zinc metal consists in allowing the ore-tubes to be made of any dimensions required for profitable operation, either in height, length, or breadth, and in providing for the free escape of the vapor without the necessity of passing it through a large mass of ore, and for its subsequent collection in either of the forms desired.

The tubes F F and M M, when used in a puddling-furnace exposed to the full intensity of the heat therefrom without any intervening roof, will require to be of fire-brick; but in most other cases they may be of metal, if for any reasons it may be desirable.

I do not claim to have invented any mode of treating the oxides or other substances after they are evaporated; but

What I do claim as my invention, and desire to secure by Letters Patent, is—

1. The combination of any number of ore-tubes F F, and tubes or spaces M M, placed side by side and communicating with each other through openings f f in their sides, the ore-tubes being exposed to a degree of heat sufficient to evaporate the oxides or other substances contained therein and make them pass through the openings f f into the tubes or spaces M M, the said tubes or spaces M M being protected from the heat by the ore-tubes, and serving either to collect and condense the oxides or other vapors or to convey them to any other suitable receptacle, substantially as herein set forth.

2. The hood or trunk N, furnished with suitable openings for the admission of air, and placed over the ore-tubes F F or spaces M M, substantially as described, for the purpose of receiving, leading off, and cooling the oxides or other vapors escaping from the ores, substantially as described.

JAS. RENTON.

Witnesses:

EL. POLHAMUS,  
O. D. MUNN.